

1

2,914,910

## PROPYL NITRATE MONOFUEL AND METHOD OF USE WITH NICKEL SALTS

Charles H. King, Jr., Manchester, Conn., assignor to United Aircraft Corporation, East Hartford, Conn., a corporation of Delaware

No Drawing. Application October 11, 1954  
Serial No. 461,645

14 Claims. (Cl. 60—35.4)

The present invention relates to an improved monofuel or mono-propellant for reaction motors, rockets, jet-propulsion motors, as well as other jet-propelled devices.

The term "jet-propulsion devices," as used herein, relates to devices which derive their driving power from the escape through a jet or nozzle at relatively high velocity of the mass comprising the products resulting from a combustion or exothermic decomposition of a fuel. The jet may be exhausted into the open air as in the rocket type of device, or it may be directed on a movable object as in the turbine type of device.

Propyl nitrate is known to be a useful monofuel or mono-propellant for jet-propulsion devices as evidenced by the prior patent to Doumani et al., 2,645,079. The term "propyl nitrate" as used herein relates to both normal propyl nitrate and isopropyl nitrate which are chemical isomers. In using propyl nitrate as a monofuel, as for example, in a jet-propulsion motor, it is charged into a feed tank and pressured with an inert gas, such as nitrogen. The fuel is pressured by the inert gas contained in a second tank under high pressure, as for example, 1500 p.s.i., through suitable lines and a pressure reducing control valve. The pressured propyl nitrate is then released from the fuel tank and fed through suitable lines and control valves through an ejector or atomizer into a combustion chamber. In the combustion chamber, the propyl nitrate is ignited by suitable means and allowed to decompose or burn.

The paramount disadvantage of propyl nitrate as a monofuel is that a large combustion chamber is required to decompose it. This is undesirable, particularly in aircraft, where lightness in weight is so essential and available space is often at a premium.

An object of my invention is to provide catalytic means whereby a smaller combustion chamber may be employed for decomposing propyl nitrate than has heretofore been possible. It is also a further object of my invention to provide catalytic means to improve the starting characteristics and combustion efficiency of propyl nitrate as a mono-propellant.

I have discovered that the foregoing objects may be accomplished by the addition to propyl nitrate of a soluble nickel salt which decomposes when heated in the combustion chamber to give finely divided nickel particles throughout said chamber in a uniform manner. These nickel particles function as a catalyst for the decomposition of propyl nitrate. Advantageously, therefore, the nickel particles formed on decomposition are uniformly dispersed throughout the chamber to catalyze effectively the decomposition of the fuel. It is not convenient to obtain this uniform dispersion of nickel particles in the combustion chamber by merely feeding nickel particles from an outside line to the combustion chamber since this would require a mechanism to inject and disperse a stream of metal particles in the combustion chamber against the high combustion pressure. Merely introducing the metal particles and the propyl nitrate fuel

2

as a slurry would also be disadvantageous as the presence of the catalytic metal surface would tend to make the fuel less stable to decomposition and more subject to explosions in the fuel lines before introducing it into the chamber. On the other hand, with the nickel salt added to the fuel according to my invention, the salt is not converted into the active metal catalyst until the fuel is in the combustion chamber. This has the advantage that the stability characteristics of the fuel will be unaffected during storage and in the feed lines to the combustion chamber.

Examples of suitable nickel salts which may be used in accordance with the present invention are nickel carbonyl, nickel acetyl acetonate, nickel diisopropylthiocarbamate and nickel dinormalpropylthiocarbamate.

Generally, the salt, calculated as metallic nickel, is in an amount from 0.02 to 1.0 percent by weight of the propyl nitrate and preferably from 0.1 to 0.25 percent by weight.

Comparison tests have been conducted which show the superior results obtained by the addition of a soluble nickel salt compared to pure propyl nitrate or for propyl nitrate with salts of other metals as shown in Table I. For example, there is an increase of specific impulse (*Isp*) to 167 sec. when normal propyl nitrate, containing 0.725 percent nickel carbonyl by weight (0.25 percent Ni) is decomposed in a chamber with a characteristic length (*L*<sup>\*</sup>) of 430 inches compared to marginal operation at a specific impulse at 145 sec. for the same chamber using pure normal propyl nitrate. Since 167 sec. is the theoretical specific impulse for the test conditions—a chamber pressure of 300 p.s.i. and normal atmospheric pressure exhaust, this corresponds to an increase in combustion efficiency from 87 to 100%. Since this concentration of nickel carbonyl in normal propyl nitrate also produced essentially 100% combustion efficiency when the characteristic length (*L*<sup>\*</sup>) of the combustion chamber was reduced to 315 inches, further reduction in characteristic length is obtainable using this catalyst-fuel mixture. The characteristic length *L*<sup>\*</sup> is the ratio of the combustion chamber volume to the exhaust nozzle throat area in consistent throat area in consistent units and is a measure of the volume required for combustion which is essentially unaffected by the scale of the rocket or combustion chamber. The particular tests related were accomplished using cylindrical combustion chambers of approximately 40 lbs. thrust requiring a fuel flow of about 0.25 lb. of propyl nitrate per sec. The combustion chamber with a characteristic length of 430 inches was 3 inches in diameter and 5½ inches long and exhaust nozzle throat area was approximately 0.09 sq. in. Additional tests in Table I were accomplished in a chamber identical in cross section and throat area but only 4 inches long (*L*<sup>\*</sup>=315 inches).

The results obtained by using the soluble nickel salts are not only advantageous but are surprising. For example, chromium acetyl acetonate, which is an effective catalyst for the decomposition of a similar mono-propellant, namely, nitromethane, did not increase the rate of decomposition of normal propyl nitrate as shown in Table I.

In order to describe my invention even further, data on the decomposition of normal propyl nitrate containing four different nickel salts are presented in Table I. As can be seen, specific impulse and combustion efficiency were increased from 4.2 to 20.2% by the addition of varying amounts of these salts.

In addition, to show that all metal salts do not have the same desirable catalytic effect on the decomposition of normal propyl nitrate, further data are presented in Table I. These data show that salts of iron, lead, cobalt

Table I

|                                         | Chamber<br>L* in. | Com-<br>ound in<br>Solution | Metal in<br>Solution | Isp<br>Without | C*<br>Without | Isp with<br>Compound      | C* with<br>Compound | Percent<br>Increase |
|-----------------------------------------|-------------------|-----------------------------|----------------------|----------------|---------------|---------------------------|---------------------|---------------------|
| Nickel Acetyl Acetonate.....            | 315               | 0.21                        | 0.048                | 144            | 3,310         | 153                       | 3,520               | 6.2                 |
|                                         | 315               | 0.44                        | 0.10                 | 141            | 3,240         | 153                       | 3,520               | 7.8                 |
| Nickel diisopropylthiocarbamate.....    | 315               | 0.21                        | 0.03                 | 140            | 3,220         | 148                       | 3,400               | 5.7                 |
| Nickel dinormalpropylthiocarbamate..... | 315               | 0.28                        | 0.04                 | 142            | 3,270         | 148                       | 3,400               | 4.2                 |
|                                         | 315               | 1.05                        | 0.182                | 140            | 3,220         | 149                       | 3,430               | 6.4                 |
|                                         | 315               | 0.145                       | 0.05                 | 143            | 3,290         | 154                       | 3,540               | 7.7                 |
|                                         | 315               | 0.29                        | 0.10                 | 143            | 3,290         | 161                       | 3,700               | 12.5                |
| Nickel carbonyl.....                    | 315               | 0.725                       | 0.25                 | 144            | 3,310         | 173                       | 3,970               | 20.2                |
|                                         | 430               | 0.29                        | 0.10                 | 144            | 3,310         | 161                       | 3,700               | 12.5                |
|                                         | 430               | 0.725                       | 0.25                 | 145            | 3,340         | 167                       | 3,850               | 15.2                |
|                                         | 430               | 2.90                        | 1.00                 | 145            | 3,340         | 172                       | 3,940               | 19.6                |
| Tetraethyl lead.....                    | 430               | 2.0                         | 1.28                 | 145            | 3,340         | 139                       | 3,200               | -4.1                |
|                                         | 430               | 2.0                         | 1.28                 | 145            | 3,340         | 139                       | 3,200               | -4.1                |
|                                         | 430               | 0.57                        | 0.06                 | 148            | 3,400         | 149                       | 3,430               | 0.7                 |
|                                         | 750               | 1.91                        | 0.20                 | 118            | 2,720         | 117                       | 2,690               | -0.8                |
| Cobalt napthenate (Note 1).....         | (Note 2)          |                             |                      |                |               |                           |                     |                     |
|                                         | 430               | 1.91                        | 0.20                 | 144            | 3,310         | 145                       | 3,340               | 0.7                 |
|                                         | 430               | 4.76                        | 0.50                 | 145            | 3,340         | 138                       | 3,170               | -4.8                |
| Iron pentacarbonyl.....                 | 430               | 4.75                        | 1.35                 | 145            | 3,340         | No data (nozzle clogging) |                     |                     |
| Carbon Disulphide.....                  | 430               | 2.0                         | 0.57                 | 145            | 3,340         | 121                       | 2,780               | -16.5               |
| Ferrocene.....                          | 430               | 0.5                         | 0.14                 | 145            | 3,340         | 146                       | 3,360               | 0.7                 |
| Chromium acetyl acetonate.....          | 430               | 2.0                         |                      | 145            | 3,340         | 145                       | 3,340               | 0                   |
| Water.....                              | 430               | 0.25                        |                      |                |               |                           |                     |                     |

NOTE 1.—Nuodex cobalt napthenate with solvent, 10.5% cobalt by weight.

NOTE 2.—150 lb. thrust chamber. All other chambers produced approximately 40 lb. thrust.

and chromium, when dissolved in normal propyl nitrate, do not promote the decomposition of the fuel. From the data of Table I, the decomposition actually appears to be inhibited as shown by decreases in specific impulse when salts of these metals are added to the normal propyl nitrate.

Standard parameters used to measure rocket performance and mentioned in the text and Table I are defined as follows in Table II below:

Table II

(1) Specific impulse as determined by thrust—

$$\text{Specific impulse} = \text{thrust}/\text{fuel flow}$$

(2) Specific impulse as determined from chamber pressure—

$$\text{Specific impulse} = \frac{P_e f_i C_f}{W}$$

where

 $P_e$ =chamber pressure $f_i$ =exhaust nozzle throat area $W$ =fuel flow $C_f$ =thrust coefficient expressed by

$$C_f = \lambda C_D \phi \Omega \sqrt{\frac{2\gamma}{\gamma-1}} \sqrt{1 - \left(\frac{P_c}{P_e}\right)^{\frac{\gamma-1}{\gamma}}}$$

where

 $\lambda$ =nozzle divergence coefficient $C_D$ =nozzle discharge coefficient $\phi$ =velocity coefficient

$$\Omega = \sqrt{\gamma} \left(\frac{2}{\gamma+1}\right)^{\frac{\gamma+1}{2(\gamma-1)}}$$

 $P_e$ =ambient atmospheric pressure $P_c$ =combustion chamber pressure $\gamma$ =ratio of specific heats(3) Characteristic velocity,  $C^*$ , as determined from chamber pressure and fuel flow—

$$C^* = \frac{P_e f_i g}{W}$$

where

 $P_c$ =chamber pressure $f_i$ =exhaust nozzle throat area $g$ =gravitational constant $W$ =fuel flow rateThe theoretical  $C^*$  may be expressed by the equation

$$C^*_{th} = \frac{\sqrt{\gamma g R T / M}}{\gamma \left(\frac{2}{\gamma+1}\right)^{\frac{\gamma+1}{2(\gamma-1)}}$$

where

 $\gamma$ =ratio of specific heats $g$ =gravitational constant45  $R$ =universal gas constant $T$ =combustion chamber temperature $M$ =average molecular weight

By utilizing my invention, smaller combustion chambers are required due to the improvement in the decomposition of propyl nitrate. Hence, lighter combustion chambers may be used, which is particularly advantageous for aircraft.

The invention in its broader aspects is not limited to 55 the specific processes and steps described but departures may be made therefrom within the scope of the accompanying claims without departing from the principles of the invention and without sacrificing its chief advantages.

I claim:

60 1. An improved monopropellant composition for use in jet propulsion devices consisting essentially of propyl nitrate and a nickel salt soluble in said monopropellant and in an amount from about 0.02% to about 1% by weight calculated as metallic nickel of said propyl nitrate, 65 said nickel salt on decomposition yielding finely divided nickel particles.

2. An improved monopropellant composition as defined in claim 1 wherein the soluble nickel salt is an amount from 0.1 to 0.25% by weight of the propyl nitrate, calculated as metallic nickel.

70 3. An improved monopropellant composition as defined in claim 1 wherein the soluble nickel salt is selected from the group consisting of nickel carbonyl, nickel acetyl acetonate, nickel diisopropylthiocarbamate and 75 nickel dinormalpropylthiocarbamate.

4. An improved monopropellant composition as defined in claim 3, wherein the soluble nickel salt is nickel carbonyl.

5. An improved monopropellant composition as defined in claim 3, wherein the soluble nickel salt is nickel acetyl acetonate.

6. An improved monopropellant composition as defined in claim 3, wherein the soluble nickel salt is nickel diisopropylthiocarbamate.

7. An improved monopropellant composition as defined in claim 3, wherein the soluble nickel salt is nickel dinormalpropylthiocarbamate.

8. A novel method for decomposing propyl nitrate monopropellant in a combustion chamber of a jet propulsion device comprising adding to said propyl nitrate outside of the combustion chamber a nickel salt soluble in said propyl nitrate and in an amount from about 0.02% to about 1% by weight calculated as metallic nickel of propyl nitrate, passing the propyl nitrate and soluble nickel salt to the combustion chamber, converting said nickel salt into finely divided nickel particles and decomposing the propyl nitrate in the presence of said nickel particles dispersed throughout.

9. The method as defined in claim 8, wherein the soluble nickel salt is added in an amount from 0.1 to 0.25% by weight of the propyl nitrate calculated as metallic nickel.

10. The method as defined in claim 8, wherein the soluble nickel salt is selected from the group consisting of nickel carbonyl, nickel acetyl acetonate, nickel diisopropylthiocarbamate and nickel dinormalpropylthiocarbamate.

11. The method as defined in claim 10, wherein the soluble nickel salt is nickel carbonyl.

12. The method as defined in claim 10, wherein the soluble nickel salt is nickel acetyl acetonate.

13. The method as defined in claim 10, wherein the soluble nickel salt is nickel diisopropylthiocarbamate.

14. The method as defined in claim 10, wherein the soluble nickel salt is nickel dinormalpropylthiocarbamate.

#### References Cited in the file of this patent

##### UNITED STATES PATENTS

|           |                  |               |
|-----------|------------------|---------------|
| 2,560,542 | Bartleson et al. | July 17, 1951 |
| 2,645,079 | Doumani et al.   | July 14, 1953 |
| 2,690,964 | Maisner          | Oct. 5, 1954  |

##### OTHER REFERENCES

- Chemical & Engineering News, vol. 26, No. 39, Sept. 25 1948, pages 2892, 2893.  
 Gunn, "Journal of the American Rocket Society," No. 22, Jan.-Feb., 1952, pages 33-38.